

R. E. KREHER.

PROCESS OF MAKING LEAD SULFATE PIGMENT.

APPLICATION FILED APR. 23, 1917.

1,248,501.

Patented Dec. 4, 1917.



Witnesses:

Edgar T. Farmer.

Amotolcombe.

Inventor:

Robert E. Kreher,  
by ~~Conrad~~ ~~Conrad~~  
his attorney.

# UNITED STATES PATENT OFFICE.

ROBERT E. KEEHER, OF COLLINSVILLE, ILLINOIS, ASSIGNOR TO ST. LOUIS SMELTING & REFINING COMPANY, OF ST. LOUIS, MISSOURI, A CORPORATION OF MISSOURI.

## PROCESS OF MAKING LEAD-SULFATE PIGMENT.

1,248,501.

Specification of Letters Patent.

Patented Dec. 4, 1917.

Application filed April 23, 1917. Serial No. 163,788.

To all whom it may concern:

Be it known that I, ROBERT E. KEEHER, a citizen of the United States, and a resident of the city of Collinsville, in the county of Madison and State of Illinois, have invented a certain new and useful Improvement in Processes of Making Lead-Sulfate Pigment, of which the following is a specification.

This invention relates to the sublimation process of manufacturing pigment composed of lead sulfate and lead oxid from lead bearing materials, such as the oxids, sulfid and carbonate of lead, described in the patents to Bartlett, No. 515,039 and No. 515,040, dated February 20, 1894.

In the process as heretofore practised, the fuel, flux and lead bearing materials are charged into a low cupola blast furnace and heated white hot, whereupon finely divided galena ore is scattered over the furnace charge and volatilized by the heat. The furnace gases are passed through a system of cooling towers and ducts, where particles of unconsumed fuel and foreign matter settle out, and the lead vapors are condensed and are separated from the permanent gases by screening. In this process about half of the lead in the charge is smelted and tapped off from the furnace into pigs, by this much diminishing the capacity of the furnace to produce pigment; because heretofore it has been necessary to melt the pigs and oxidize them into litharge before they could be charged back into the pigment furnace.

The objects of the invention are to increase the output of pigment produced in each furnace and to improve the quality of the pigment, without using any more fuel than heretofore.

The invention consists in adding to the furnace charge, as a substitute for litharge and other lead bearing materials, a considerable amount of metallic lead in the form of irregular flakes or little balls of thin crinkled metal resembling pop corn in size and appearance.

Suitable apparatus for carrying out the invention is illustrated in the accompanying drawings, the operation of which is described below; and what is claimed as the invention appears from the appended claims.

In the drawings,

Figure 1 is a side elevation of the furnaces and cooling apparatus for producing

pigment, one of the furnaces being shown in section in order to disclose the materials and their arrangement in the furnace; and

Fig. 2 is a vertical cross-section through apparatus for making flaked lead suitable for use in the process. The pigment producing apparatus comprises two similar low cupola blast furnaces 11, which are arranged side by side and discharge their gaseous products through a water-jacketed flue 12 into a large receiving tower 13. From the receiving tower the hot gases pass through a series of cooling and settling towers 14 and pipes 15, wherein particles of unburned fuel and other undesirable solid matter settle out, and the lead fumes are condensed in the form of white powder. The gaseous products and fine metallic particles are drawn out by a fan 16 and forced into a system of dust collectors (not shown), from whence the carbonic acid gas and sulfur dioxide escape into the air leaving behind the condensed metallic particles, which resemble fine white flour in appearance.

The flaked lead, lead bearing materials, coke and lime stone or other flux in the furnace charge, are shoveled into the furnaces in layers through the charging openings 17, and the slag and molten lead produced are tapped off at the bottom of the furnace through suitable tap holes 18. A blast of air is constantly blown into the furnace through the tuyers 19 for maintaining a rate of combustion suitable for producing the necessary furnace heat. About 2000° Fahrenheit is found to be a suitable temperature in the flues immediately over the furnaces. Galena ore (lead sulfid) in finely divided form is sprinkled over the furnace from time to time, and is volatilized by the intense heat and carried into the flue with the heated products of combustion of the furnace charge.

Flaked lead suitable for use in the process is prepared by melting pig lead in a pot or kettle 21, from which it is permitted to flow into a suitable receptacle 22 from whence it falls continuously in large drops or small streams. A stream of water 23 from a suitable tank 24 is directed against the falling lead and breaks up the lead into flaky masses, which are carried with the water into a tank 25. In the bottom of the tank 25 there is a conveyor 26 for removing the lead flakes to a waiting car 27 as fast as they

are formed. Other means of flaking the lead may be devised, and this invention is not restricted to this particular method or apparatus.

5 I claim the following as my invention:

1. The process of making white lead pigment which comprises heating lead bearing materials and metallic lead in the form of flakes together with flux and fuel in a blast furnace, and collecting and condensing the vapors produced, substantially as described.

10 2. The process of making white lead pigment which comprises heating lead bearing materials and metallic lead in the form of flakes together with flux and fuel in a

blast furnace, collecting and condensing the vapors produced, and tapping off the pig lead for re-charging into the furnace.

15 3. The process of making white lead pigment which comprises heating lead bearing materials and metallic lead in the form of flakes together with flux and fuel in a blast furnace, collecting and condensing the vapors produced and tapping off the pig lead, 20 melting the pig lead and dropping it into a stream of water to flake it for re-charging into the furnace.

25 Signed at Collinsville, Illinois, this 19th day of April, 1917.

ROBERT E. KREHER.